

No. 643,096.

Patented Feb. 6, 1900.

S. B. CHRISTY.

**PROCESS OF RECOVERING GOLD AND SILVER FROM CYANID SOLUTIONS  
BY ELECTROLYSIS.**

(Application filed Feb. 9, 1898.)

(No Model.)

Fig. 1.



Fig. 2.



Fig. 3.



## Witnesses.

Hellontenverde

Walter F. Vane.

## Inventor

Samuel B. Christy,  
by Gen'l F. Booth,  
his Attorney.

# UNITED STATES PATENT OFFICE.

SAMUEL B. CHRISTY, OF BERKELEY, CALIFORNIA.

## PROCESS OF RECOVERING GOLD AND SILVER FROM CYANID SOLUTIONS BY ELECTROLYSIS.

SPECIFICATION forming part of Letters Patent No. 643,096, dated February 6, 1900.

Application filed February 9, 1898. Serial No. 669,615. (No specimen.)

*To all whom it may concern:*

Be it known that I, SAMUEL B. CHRISTY, a citizen of the United States, residing at Berkeley, in the county of Alameda and State of California, have invented certain new and useful Improvements in Electrolytic Recovery of Gold and Silver from Cyanid Ore-Extraction Solutions; and I do hereby declare the following to be a full, clear, and exact description of the same.

My invention relates to the metallurgy of the precious metals, and more particularly to the electrolytic precipitation of gold and silver from the large volumes of dilute solutions of alkaline cyanids which result from the extraction of gold and silver ores, tailings, concentrates, and similar products. Such solutions are usually very dilute and offer great resistance to the passage of the electric current. Hence electrodes, large in area and great in number, must be employed to reduce the electric resistance of the solution and to render the operation practicable; but this creates another difficulty quite as serious—namely, the deposited gold is distributed over an enormous area and in an extremely thin film. To make clear the serious nature of this difficulty, I cite the following as an example: I suppose an electrolytic cell or deposition-box containing sixty-one anode and sixty cathode plates, each of ten square feet, or, counting both faces of each cathode, twenty square feet, of effective surface for each cathode, or in all a total of twelve hundred square feet of cathode area for the sixty cathodes. In such a cell an electrodeposition of six hundred ounces gold per month would be regarded as a large output. Now six hundred ounces of gold distributed over an area of twelve hundred square feet of cathode would make a film only 0.00034 of an inch or about one three-thousandth of an inch thick. When it is remembered that such a cell often has a cathode area of double what I supposed to deposit less than two hundred troy ounces per month, it must be evident that the thickness of the gold film will not in this case exceed one twenty-thousandth of an inch in thickness. It must then be evident how serious is the nature of the difficulty which remains after the gold is deposited from these dilute ore solutions in a thin film on the cath-

odes. The precious metal still remains to be recovered from a surface of from twelve hundred to two thousand four hundred square feet of cathode.

In order to make clear the advantages of my invention, it is only necessary to briefly consider the methods now in use to recover this thin film of gold from the cathodes. Among these the most prominent may be mentioned that of Siemens and Halske, where the gold is deposited on sheets or shavings of lead, which act as cathodes. On these are deposited during the month from six to eight ounces of gold to every one hundred ounces of lead. Hence when the clean-up is made at the end of the month an amount of lead from twelve to sixteen times as great as that of the gold has to be burned or cupelled off in the cupellation-furnace. This is an expensive and unsatisfactory method of recovering the gold from the cathodes, though it is at the present time probably the best in use.

In another prominent method—that of Petlan-Clerici—the gold is electrically deposited in a mass of quicksilver many times greater in weight than the gold. From the quicksilver the gold can be recovered only after the tedious and unsatisfactory operations of filtering, straining, retorting, and melting.

In the Keith process, recently introduced, the gold is precipitated with quicksilver as an amalgam on cathodes of copper or iron. From the enormous area of twelve hundred to two thousand four hundred square feet of cathode the amalgam must be recovered by the tedious and imperfect process of scraping followed by retorting and melting.

Still another method, the Bettel process, recently introduced in South Africa, is to precipitate the gold electrolytically on zinc shavings, from which the zinc is subsequently removed by dissolving it in a stronger solution of cyanid of potassium containing gold.

The large number of methods that have been devised for recovering the gold from the cathodes after it has been deposited upon them from the solution is the best proof that this difficulty has not yet been overcome.

It is the object of my invention to avoid all the difficulties that come from the handling of added base metals—such as lead, copper,

quicksilver, or zinc—and to produce a pure article of gold or silver, or both combined, alloyed only with traces of such metals as may be accidentally contained in the cyanid solution, being simultaneously extracted by it from the ore with the gold and silver. By avoiding an excessive tension at the electrodes of the cell the precipitation of these impurities with the gold and silver may also to a large extent be avoided.

Briefly stated, my process is a process of progressive electro concentration and recovery of the extremely minute traces of gold and silver contained in the dilute cyanid solutions which result from the extraction of gold and silver ores, concentrates, and tailings.

My process consists, first, in the electrodeposition of gold and silver contained in such dilute solutions upon removable cathodes sufficiently numerous and large in area to secure efficient deposition; second, in stripping and concentrating the thin film of gold and silver thus distributed over a large number and area of cathodes in a smaller volume of cyanid solution by suitable means. These means for stripping are, in preference, electrolytical by making the gold-laden cathodes in turn anodes in the smaller volume of cyanid solution; but the stripping may also be accomplished by the action of a smaller volume of cyanid solution containing suitable oxidizing agents, and, third, in precipitating the gold contained in this smaller volume of enriched cyanid solution electrolytically upon a smaller number of cathodes, preferably upon one cathode. In general I prefer to perform the second and third operations simultaneously; but they may also be separately performed. These general steps, together with all necessary details of apparatus and manipulation, will be more fully understood from the following description and by reference to the accompanying drawings, designed to illustrate generally an apparatus suitable to the purpose.

In the drawings, Figure 1 is a vertical longitudinal sectional view of what I may term the "deposition-box." It is an ordinary electro-deposition-cell in which the gold and silver are precipitated from the dilute ore solution and distributed over the enormous area of the cathodes necessary for effective deposition. Fig. 2 is a similar sectional view at right angles to the planes of the electrodes of what may be termed the "finalstripping and concentration box," or simply the "clean-up box" for the purpose of finally concentrating the gold spread out over a large number of cathodes upon a single cathode. Fig. 3 is a similar section of an "intermediate stripping and concentration box."

In Fig. 1, B represents a water-tight box provided with grooves on the longitudinal sides to receive the electrodes A and C. The anode-plates, (marked A,) beginning at the head of the box, are each slipped into alternate

grooves and rest in the bottom grooves. The top of the anode-plates A must be below the water-line an inch or more. The anode-plates are all placed in suitable electrical connection with the positive pole of a shunt-wound dynamo or other external source of electric energy. The anodes are thus connected in parallel. In the alternate grooves between the anodes are now slipped the cathodes, (marked C.) These reach above the surface of the solution and within about an inch or more of the bottom of the cell, and the cathodes are similarly placed in electrical connection with the negative pole of the same shunt-wound dynamo or other external source of electric energy. I have not thought it necessary to encumber the drawings with the details of these connections, as they are well understood, deeming it sufficient to mark the anodes with a plus sign and the cathodes with a minus sign. The ore solution enters at the head of the deposition-box at D and passes down between the first anode and cathode, up between the first cathode and second anode, and so on alternately up and down in the direction of the arrows till it finally leaves the tail of the box at E. If desired, the circulation of the solution may be equally controlled by having the cathodes reach to the bottom of the box and so as to be immersed below the surface of the solution at the top, while the anodes are lifted above this bottom and above the solution at the top; but in general I prefer the former arrangement. Both electrodes, and in particular the cathodes, are made so that they can be readily removed one or more at a time from the cell without disturbing its operation. The anodes and cathodes may be made of any electroconducting material not too strongly acted on by the solution, such as lead or iron; but usually on account of its cheapness I prefer to make them both of wrought-iron, the anodes about an eighth of an inch or less in thickness and the cathodes as thin as they can be made without buckling.

As my claim is for a process and not for a particular form of apparatus, I do not wish to be understood as confining myself to the particular form of deposition-box here described. Any form of electrolytic cell may be used in which the gold and silver bearing solution is brought into progressive contact with removable cathodes sufficiently numerous and large in area to secure efficient deposition.

In Fig. 2 is shown a vertical section of the final stripping and concentration box or the clean-up box, taken at right angles to the plane of the electrodes. F is a water-tight box of non-conducting material and containing, preferably, two anodes II II, supposed to be connected in parallel with the plus or positive pole of a shunt-wound dynamo or other external source of electric energy, and preferably a single cathode, (marked G,) supposed to be connected with the negative pole of the same source of electric cur-

rent as the anodes H H. Both anodes are made so that they can be removed one at a time from the box F without interfering with the passage of the current. The cathode G 5 is also removable. The anodes H H in the clean-up box F are the gold or silver laden cathodes C C from the deposition - box B, which are to be stripped of the film which has been deposited upon them. The cathode 10 G in the clean-up box F may be made of any suitable electroconducting material; but in preference I use an extremely thin sheet or series of thin strips of gold or silver of suitable area. This general description will suffice 15 to explain the process carried out in such an apparatus. The solution to be precipitated as it comes from the extraction of an ore is a double cyanid of gold and silver and an alkali, such as potassium, together with 20 some cyanids of the base metals, also removed by the solution from the ore. The solution should be decidedly alkaline, and if it is not already should be made so by the addition of caustic potash, soda, or lime. Between the 25 anodes and cathodes, each connected in parallel, I now maintain a constant electrical potential, preferably between one and a half and two volts, though I do not confine myself to these tensions. The proper tension is en- 30 tirely dependent on the amount of free cyanid present. If the amount of free cyanid is low in proportion to the gold present, lower tensions than one and a half volts will suffice; but if there is a relatively large amount of 35 free cyanid present in proportion to the gold higher tensions, such as two and a half to three volts, are necessary to get a high extraction of the gold; but I prefer not to use these high tensions unless absolutely necessary, as they lead to large consumption of 40 the cyanid used. I prefer to work with the lowest tension possible and to increase the precipitation by increasing the cathode area rather than the tension. With a constant 45 electrical potential at the electrodes and a given strength in free cyanid the rate of precipitation of the gold is fixed by the gold content of the solution, by the number and area of the electrodes, their distance apart, and 50 the rate of flow of the solution through the box. The electrodes should be as numerous and as near together as practicable without causing short-circuiting. A distance of an inch or an inch and a half is usually as close 55 as it is safe to place them in practice, owing to danger of buckling; but if vertical strips of wood are fastened to the anodes at intervals of about a foot apart the electrodes may be placed as near together as half an inch 60 without danger from buckling. When the gold and silver content of the solution has been sufficiently reduced, it is discharged from the deposition-box B, and after being sufficiently reinforced with cyanid it is again 65 ready to extract a new portion of ore, and so on indefinitely. The gold may be almost entirely removed from the solution in the

deposition - box B if sufficient time is given; but the first three-fourths of the gold and silver are much more quickly removed than the 70 last fourth, and as the solution is used over and over again it is usually best to shorten the time of the treatment by precipitating only about three-fourths of the gold contained in the solution as it enters the box. Now, as 75 the solution flows through the box B with a constant tension at its electrodes, the electric current at the head of the box will be greater than at its tail, because more gold is contained in the solution as it enters than as it leaves 80 the box, and the cathodes at the head of the box will become more rapidly covered with gold than those at the tail end of the box, where the gold has been more reduced. As the cathodes at the head of the box become 85 coated with gold I remove them successively in pairs from the head of the deposition-box B and make them anodes in the clean-up box F. Of the cathodes C C remaining in the deposition-box B, I prefer to move them step- 90 wise from their places up toward the head of the box, and in the place of those left vacant at the tail end of the box I insert other cathode-plates that have just been stripped of their gold content as anodes in the clean-up 95 box F, and so on in endless course.

In order to make more clear the advantages of my method over those now in use and without confining myself to the numbers and dimensions here given merely in illustration, I will suppose the case cited in the introduction—viz., an electrolytic deposition-cell with sixty cathode-plates with a total effective cathode area of twelve hundred square feet is producing, say, six hundred troy 100 ounces of gold per month of thirty days. In this case, if it were required to make a monthly clean-up, I would proceed as follows: Every day I would take two of the original cathode-plates C C from the head of the deposition-box B, and they would be removed to the clean-up box F. I would then move from the tail of the deposition-box toward its head the remaining cathodes C C, and in place of the spaces left vacant at the foot of this box 110 I would insert two cathodes C C that had just been anodes H H in the box F and had just been stripped of their gold content. In this way a pair of original cathode-plates C C 115 would go every day to the clean-up box F. This cell would contain a solution of an alkaline cyanid. As this solution is used over and over again continuously and as it is comparatively small in volume, it may be conveniently made without undue expense slightly 120 stronger in cyanid than the original ore solution; but this extra strength is not usually necessary, and the solution should not be made too strong in cyanid, for then while it strips the gold very rapidly from the anodes it becomes 125 extremely difficult to redeposit the gold from it upon the cathode. The pair of original cathodes C C from the box B are made to replace the already-stripped anodes H H in the 130

clean-up box F and are themselves made anodes H H in the box F. From the sides of the anodes H H turned toward the secondary cathode G the gold is rapidly stripped by the electric current, and unless the cyanid solution is made too strong an equal amount is deposited on the secondary cathode G. The current should be so graduated that it is deposited on G in a firm coherent coat. If a very strong current is used, the gold is deposited on the cathode G as a fine brown powder, which may be brushed off at intervals and melted down; but I prefer to deposit it as a firm coherent coat to avoid mechanical loss in handling. As soon as the gold is stripped from one side of the plates H H the other side of each plate is turned toward the cathode G and this side of each plate is stripped in like manner. After being sufficiently stripped of their gold deposit in the clean-up box F the anodes H H are again made cathodes C C in the deposition-box B to receive a new deposit of gold, as before.

While it is desirable to strip the gold from the anodes H H in the clean-up box F as completely as possible at each operation, it is not absolutely necessary to do so, for what is not recovered at one operation will be recovered at the next, as the same plate is alternately cathode C in the box B and anode H in the box F.

Owing to the fact that the gold dissolved from the anodes H H furnishes as much energy as is required to deposit the same amount of gold on the cathode G and as on account of the small volume of the solution in the clean-up box it may without undue expense be made slightly stronger in cyanid than that in the deposition-box B, it follows from either or both of these two causes that the same electromotive force at the dynamo will produce a denser current and the plates H H will be usually stripped clean of their gold in much less than twenty-four hours, so that all the gold deposited in thirty days' slow work on the two electrodes H H (called C C when in the box B) is in one day transferred to the single plate G. By repeating this process daily for thirty days at the end of the month all the gold deposited in thirty days on both sides of the sixty cathodes in the deposition-box B has been transferred in the clean-up box to the single cathode G. Thus in the case cited instead of having at the end of the month six hundred troy ounces of gold distributed over an area of twelve hundred square feet in a film one three-thousandth of an inch thick it is concentrated in a single sheet of not more than ten square feet and not less than one twenty-fifth of an inch in thickness. In such a state it is not necessary to melt it into bars. All that is left to be done is to cut it into sheets of a suitable size for transportation to the mint. Hence without the intervention of an expensive and complicated auxiliary plant entirely foreign in nature and operation to that used in depositing the gold from the ore

solution and by the use of very simple appliances in harmony with the rest of the process I am able to turn out my monthly product 70 of gold and silver at a nominal extra expense nearly pure and ready for the mint.

In case it has been necessary to use two thousand four hundred square feet instead of twelve hundred square feet of cathode-surface in the deposition-box B the advantage of my process over the usual methods is even more apparent. It should be further remarked that while after stripping the anodes H H in the clean-up box F it is best to replace the same as cathodes C C at the bottom of the deposition-box B and to move them as they become coated with gold progressively toward the head of the box B until they are finally removed to the clean-up box F this 85 progressive rotation may be omitted and the cathodes C C may be removed, stripped, and returned in any order that may be convenient. In general in spite of the labor involved in the progressive rotation I prefer 90 it, for when the stripped cathodes C C are placed at the tail of the box they offer no back electromotive force to the current, and the solution, already low in gold at this point, is more completely deposited on the recently-95 stripped cathodes than it would be on cathodes already partly coated. It is also evident that I may modify the relative periods during 100 which any single cathode is being covered, according to the relative strengths of solutions that are being treated in the deposition-box, without in any way altering the principle and that any person skilled in the electrometallurgical art would be able to make such changes without further instructions. In 105 case, however, of an establishment operating a large number of deposition-boxes then between these boxes B B and the clean-up box F, I prefer to introduce a third box J, (shown in Fig. 3,) which I term the "intermediate 110 stripping and concentration box." The intermediate box thus introduced contains a smaller number of electrodes than the deposition-box B. These anodes K and the secondary cathodes L are all exactly like the cathodes 115 in the deposition-box B and are connected in parallel with an external source of electric energy, as in said box. In using the intermediate stripping and concentration box J the cathodes C C from the deposition-boxes 120 B B are made anodes K in the intermediate box J, and the gold is thus transferred to the cathodes L of this box. The stripped anodes K in the intermediate box J are then made cathodes C C at the tail of the deposition-boxes B B. For example, to work conveniently a plant of, say, five deposition-boxes B B there would be, say, ten anodes K K in the intermediate box J. In this way all the gold from, say, three hundred cathodes C C 125 in the five deposition-boxes B B could be concentrated on, say, eleven cathodes L L in the intermediate stripping and concentration box J. Of these eleven cathodes nine would 130

be intermittently in said intermediate box J receiving their coat of gold. Two others, meanwhile in rotation, would be made anodes H H in the clean-up box F, where their gold content would be transferred to the single sheet or final cathode G, which would thus contain at the end of the month, in the case cited, over sixty thousand dollars in a single sheet, say, ten square feet in area and one-fifth of an inch in thickness.

In very large establishments it will prove simpler to arrange the clean-up box as I have described the intermediate box with several cathodes and anodes. Only in this case the final cathodes would preferably be made of thin sheet gold or silver instead of iron.

The cathodes G in the final stripping and clean-up box, instead of being made, as I have mentioned, of gold or silver, may be made of any other metal, such as iron or lead or copper. In this case a coat of electrotyper's graphite or other similar substance is to be given to the smooth surface of the metal, so that after the gold or silver has been deposited on the same of sufficient thickness it may be peeled off in sheets and cut up or melted down, as desired.

Now, although I prefer the electrical stripping and concentration of the gold and silver in the clean-up box at a single operation, as already described, as the simplest and most efficient method I do not confine myself to this method, for the gold-laden cathodes C C from the deposition-box B may be treated

one or more at a time in a small box having in it a smaller volume of an alkaline-cyanid solution, together with some suitable oxidizing agent—such as air, peroxids of hydrogen, barium, sodium, or some other metal or ferricyanid of potassium, or permanganate of potassium. If the cathodes C C are immersed in such a solution, so that not only the gold film is immersed, but also the uncoated sheet-iron above the gold, the latter will be rapidly dissolved, particularly if the solution is gently agitated, and after stripping a large number of cathodes the enriched solution which finally begins to act slowly is precipitated as before by introducing an anode and a suitable cathode and connecting them with an external source of electrical energy, so that the gold is recovered as before in a single sheet.

I am aware that to deposit gold electrolytically upon cathodes is not new, nor do I wish to be understood as claiming it to be new to strip films of electroplated metals from electrodes in a conducting solution by electrical means, such being employed by electro-

platers to recover the gold from imperfectly-plated articles. I am also aware that British Patent No. 16,737, granted Pfleger September 6, 1895, suggests that by placing the gold-plated electrodes in a ten-per-cent. cyanid-of-potassium solution in contact with a plate of carbon the gold will dissolve and a concentrated solution will result, from which the gold may afterward be extracted. I am also aware that it is not new to strip thin gold films from imperfectly-plated articles and to redeposit this gold electrolytically upon suitable cathodes, this practice being long known to electroplaters, as shown by Wahl, p. 260, paragraph 2, where a ten-per-cent. solution of cyanid is used. None of these separate operations do I claim to be new and expressly disclaim same. However, so far as I am aware such steps have never before been combined and coördinated in a single progressive process in such manner that they constitute a common function, whereby the extremely minute traces of gold and silver (often less than one two-hundredths of one per cent.) contained in the extremely dilute cyanid solutions which result from the treatment of ores, concentrates, and tailings have been concentrated by electrolytical methods alone in a single sheet of pure metal, thus securing a concentration of more than two hundred thousand to one without resorting to any auxiliary method or operation.

What I claim, and desire to secure by Letters Patent, is—

The process of progressive electroconcentration and recovery of gold and silver contained in the large volumes of dilute cyanid solutions containing free alkali resulting from the extraction of gold and silver ores, tailings and concentrates, which consists—first, in depositing the gold and silver electrolytically from said solution upon removable cathodes sufficiently numerous and large in area to secure efficient deposition, and second, in making said removable original cathodes successively anodes in a smaller volume of cyanid solution and transferring and depositing electrolytically the thin film of gold and silver, already distributed over a large number of said original cathodes, upon a smaller number of secondary cathodes, also contained in said smaller volume of cyanid solution.

In witness whereof I have hereunto set my hand.

SAMUEL B. CHRISTY.

Witnesses:

D. B. RICHARDS,  
WALTER F. VANE.